

Feb. 9, 1937.

G. S. HIERS

2,070,335

POROUS COATED PILE FABRIC

Filed Oct. 16, 1935

*Fig. 1*



*Fig. 2*



*Fig. 3*



*Fig. 4*



*Fig. 5*



*Fig. 6*



*Inventor*

*Glen S. Hiers*

*By Paul J. Schmitz*  
*Attorney.*

## UNITED STATES PATENT OFFICE

2,070,335

## POROUS COATED PILE FABRIC

Glen S. Hiers, Bala-Cynwyd, Pa., assignor to  
 Collins & Aikman Corporation, Philadelphia,  
 Pa., a corporation of Delaware

Application October 16, 1935, Serial No. 45,357

9 Claims.

(Cl. 28—1)

My invention consists of an improved and novel pile fabric in which the loops of the pile are firmly united to a backing fabric by an insoluble solidified pliable composition which is so positioned and proportioned in the fabric that the original porosity or ventilating quality of the fabric before the application of such composition is largely retained.

More particularly, my invention resides in an improved V-pile fabric, suitable for upholstery use, in which the pile V's are looped in weaving around single wefts of a backing fabric which is composed of backing warps and wefts interwoven to form a single plane ground for the pile loops. A cementitious binder material is incorporated, substantially locally, in the backing fabric threads and that portion of the tuft which lies in the same plane. A less quantity of binder material to hold the tufts securely in place is required than in present commercial fabrics.

It is well known that this type of pile weave effects greater coverage for a given quantity of the pile yarn, which may be of wool or other animal fiber such as mohair or vegetable fibers such as cotton or combination yarns containing any two or more of these, than the W or fast pile loop and the objectionable "grinning through" of the knees of the W tufts is also avoided. As the V-pile tufts are looped about a single weft thread, it is sometimes necessary that auxiliary means be applied to or incorporated in the fabric to insure good "anchorage" of the pile tuft. The term anchorage means the resistance offered by the pile tufts to dislodgement relative to the backing fabric.

Heretofore, such auxiliary means have been applied in various ways, for example, as disclosed by the Drobile Patent No. 1,788,989 issued January 13, 1931. This patent, along with any prior art of which I am aware, deals with a method of manufacture of or a fabric in which anchorage of the pile tufts and reenforcement of the backing is obtained by means of a substantially continuous film which tends to make the finished fabric moisture-proof and hence, deficient in porosity for many purposes. It is the purpose of this invention to set forth a loose pile fabric in which the binder material is not continuous but follows and is largely confined within and on the threads and at their points of interlacing rather than in the interstices between them so as to preserve the natural porosity of the fabric and yet firmly anchor the tufts in their positions. It has been found that the anchorage of the tufts, relative to the weight of a binder material such as one containing rub-

ber can be greatly improved and hence, a porous or ventilated coated V-pile fabric can readily be produced. The amount of binder material used is dependent on the character of the woven web, that is, looseness of the weave, the materials used, etc.

Applicant knows of no standard machine for reducing the anchorage of the pile tufts to accurate mathematical terms. The usual way of determining whether or not anchorage is commercially satisfactory is for the inspector to firmly stretch the fabric with his hands and then by strongly rubbing the forefinger over the face of the pile attempt to wholly or partially dislodge the tufts through the back of the fabric. A commercial fabric of this type may be defined as one in which it is impossible or exceedingly difficult to dislodge the tufts by the method indicated.

In comparable textures of woven webs equal anchorage of the pile tufts to that obtained in prior fabrics is obtained in the present invention with greater than 20% less rubber by weight. This is because the binder is confined to its most effective positions and because there is a great increase in the number of anchoring points.

Permeability to air or porosity is a very desirable characteristic in this type of fabric in order that certain objectionable features of the fabric, when in use, may be overcome. In automobiles, for example, there is a tendency to trap air within the cushion and to produce as a result thereof an objectionable air cushioning independent of that derived from the normal cushioning structure. The ventilating property of the fabric also avoids the accumulation of heat within the fabric and hence, increases the riding comfort of the passenger.

It is an object of this invention then to provide a pile fabric having securely anchored pile V's but which is quite porous or permeable to air.

It is a further object of this invention to provide a V-pile fabric which will not act as a trap for air which may gather on the back side of it when the fabric is in use as on a seat cover or automobile upholstering cushion.

A further object of this invention is to secure the warp pile tufts firmly in their original positions with a minimum amount of binder material and to so position said binding material that both the textile feel of both sides of the fabric and the ventilating qualities of the fabric will not be destroyed.

A further object of this invention is to secure the pile tufts in such a way that they may have

a cradle action when the fabric is draped so that the softness of the face is largely retained after impregnation.

A further object of this invention is to provide a pile fabric which has been scoured, preferably locally, and to which, before the moisture has been lost by evaporation or otherwise, a binder material is incorporated in the backing thereof. The binding material is so diffused through the scoured and wetted threads that a substantial portion of the individual fibers of the different threads making up the fabric is completely covered and consequently the individual fibers act to anchor the pile tufts in position. This results in a pile fabric having an even spacing of tufts and hence, a uniform coverage on the face of the fabric.

Figure 1 is a diagrammatic bottom plan view of a fabric before impregnation.

20 Figure 2 is a diagrammatic view of the fabric shown in Figure 1 and illustrates the localizing of the impregnating matter about a single pile loop.

Figures 3 and 4 are diagrammatic sectional side and end views of a single pile loop and the impregnated backing threads of Figure 2.

Figures 5 and 6 are diagrammatic views of similar fabrics showing variations in the relative positions of the pile loops to the backing threads.

Applicant makes no claim to the several structures per se, but only when they are impregnated as set forth. The fabrics are made up of backing warps 1, 1' and 1''; backing wefts 2, 2' and 2''; and pile loops 3, 3' and 3'', respectively. Reference numeral 4 designates the anchoring material diffused throughout the length of the backing yarns and localized in the tufts so as to leave the interstices of the back substantially free of anchoring material. This, as may be clearly seen, allows for a rocking action of the pile loop about its supporting weft. It is to be understood of course that the fabric must be woven tightly enough to provide good pile coverage on the face of the fabric.

The local scouring is accomplished by applying substances to the back of the woven web, which will remove the water-repellent oils, which are normally present, from the threads and this, together with the moisture left in the fabric as a result of the scouring, apparently causes the threads to have a greater affinity for the binder material than do the interstices between the threads and hence, the interstices will not be closed unless an excessive amount of binder material is applied. The woven web may of course in some cases be wholly scoured, but local scouring is preferred as it tends to definitely restrict the binder affinity properties of the finished fabric to that portion which will actually take the binder material.

60 A suction or blower apparatus may be used to blow or draw off surplus water, which may be left on the fabric as a result of the scouring. This latter step regulates the amount of water in the fibers and removes water from the interstices between the tufts and threads, so that when the binder material is applied, it permits the binder, due to increased affinity of the wetted fibers and/or the increased capillarity of the scoured and wet yarns, to thoroughly diffuse and position itself around and into the individual fibers of the threads so that they may act to individually anchor the pile tufts. The amount of local scouring, moisture content of the fabric, and the viscosity of the binder fluid when applied are all 75 contributing factors to the positioning of the

binder material in the manner set forth. Applicant accordingly does not wish to limit himself to any specific method for attaining his result but is claiming and believes to be new, a V-pile fabric in which the pile V's are securely anchored in position by a binding material, which diffuses through and which is largely confined within the thread of the woven fabric. In this way, a securely anchored pile tuft is incorporated in a porous or ventilated fabric by means of a lesser amount of binder material than was previously possible. The fibers of the individual tufts become cemented together, as it were, and the outside fibers thereof become cemented to the fibers of the backing threads. Thus, it is seen a different type of anchorage is obtained than when a continuous or skin coating is used. This is well illustrated by dissolving out the textile material of a fabric with a continuous web of rubber binder and of a fabric with the binder material located as herein described. In the former, an impervious sheet of rubber is obtained, whereas in the latter, a decidedly flimsy, perforated sheet and in some cases just a mass or ball of rubber having no definite shape results.

25 The cradle action referred to in the objects of invention results from the position and localizing of the binder material. By confining it largely to the outline of the backing and by leaving the interstices open, a hinge action or fulcrum point is produced intermediate the extreme bottom of the pile bights and their tips. This permits lateral or filling-wise rocking movement of the bights of the pile tufts and tends to retain the softness of the face of the fabric.

30 Each pile warp thread, in this type fabric, may contain 35 or more separate and distinct fibers. It is known that in prior fabrics, only a small part of the thread area is in contact with the binder material. By so positioning the binder material, in this mechanically more effective position, rather than in the interstices of the fabric, both better anchorage and porosity of the fabric are obtained. In the present invention, the pile tuft fibers are individually set in the binder material.

35 Fabrics of similar weaves and yarn count and commercial anchorage were tested on a textile porosity testing machine as developed by the Bureau of Standards and the new fabric herein set forth showed improved porosity in the face to back direction of from 95 to 338 percent, and in the back to face direction of 55 to 110 percent.

40 By thus confining the binder material within the backing threads and the pile tufts locally to the plane of the backing material, the bights of the pile tufts are left clean and project from the plane of the binder material. The apparatus for applying the binder material may include a wiping or scraping element for the pile bights. This tends to clean them of binding material, and hence, the back of the finished fabric will retain its textile character or feel and the flexibility of the web is preserved.

45 The finish of the fabric is accordingly improved and the draping characteristics are very good. So far as appearances are concerned, the fabric closely approaches a completely textile or thread fabric.

50 The term coated is used herein to define an adhesive-bound fabric in which the binder material has been applied to anchor the tufts, and not to define a continuous imperforate film of binder material after solidification.

5

10

15

20

25

30

35

40

45

50

55

60

65

70

75

75

Applicant further wishes it to be understood that this invention does not depend on the particular binding material used, although he has found that aqueous dispersions of rubber containing vulcanizing substances or aqueous dispersions of nitrocellulose, preferably in colloidal forms, are effective after the woven web has been prepared as indicated above. Organic solutions of rubber and nitrocellulose or pyroxylin may be used as equivalents. The substances may be defined generally as normally insoluble.

My improvements are applicable to the treatment of pile fabrics woven singly or on the double plush principle and which may be woven with relatively few picks of weft threads over which pile tufts are looped. Closely woven V-pile fabric having a total measured thread area equal to 100% or more of the fabric area, may not need any binder material to anchor the tufts. Highly successful commercial V-pile fabrics of less than 100% fiber density of the fabric area, and with excellent coverage have been made with the aid of binder material as set forth.

It is pointed out, however, that because of the greater affinity of the fibers for the binding material in the fabric treated as indicated herein than in previously woven webs, the porosity of more closely woven fabrics or fabrics in which there is substantial compression between certain threads of the backing and/or the tufts, due to crowding of the threads in the reed dents or the like, will be maintained after application of the binder material and the natural flexibility of the fabric preserved. The fact that the binder is in the same plane as the backing fabric tends to effectively preserve the flexibility of the web.

The fabrics may be decorated by cutting, singeing, embossing or acid treatment in any usual way.

Having described my invention, I claim—

1. An impregnated ventilated flexible single-plane backing V-pile fabric which consists of interwoven warp and weft backing threads, warp pile V tufts having their tips free of impregnating material looped around a single weft thread so that the tips of the pile bights project below the backing threads, said pile tufts being firmly anchored in the backing fabric by a cementitious binding material, which is thoroughly diffused in and largely confined within said threads and locally to and in said tufts at that portion of the tufts which are in the plane of the backing threads, whereby the interstices between the threads are not filled and the porosity as well as the textile feel is preserved on both sides of the finished fabric.

2. An impregnated ventilated flexible single-plane backing V-pile fabric which consists of interwoven warp and weft backing threads, pile V tufts having their tips free of impregnating material looped around a single backing thread, said pile tufts being firmly anchored in the backing fabric by a normally insoluble binder composition which is thoroughly diffused in and largely confined within said threads and locally to and in said tufts at that portion of the tufts which is in the plane of the backing threads so as to provide a discontinuous layer which does not fill the interstices between the threads, whereby the porosity as well as the textile feel is largely preserved in both sides of the finished fabric.

3. An impregnated ventilated flexible single-plane backing V-pile fabric which consists of interwoven warp and weft backing threads, warp pile V tufts having their tips free of impregnat-

ing material, looped around a single weft thread and having the pile bights projecting from the backing fabric, said pile tufts being anchored in position by a discontinuous normally insoluble binder composition containing rubber, free of the interstices between the threads, and confined substantially within the perimeters of the backing threads and locally to and in said tufts at that portion of the tufts which is in the plane of the backing threads to allow a hinge action or rocking of the pile tufts and to preserve the softness and flexibility of the fabric.

4. An impregnated porous flexible single-plane backing V-pile fabric which consists of interwoven secured warp and weft backing threads, warp pile V tufts having their tips free of impregnating material looped around a single weft thread and having the pile bights projecting from the backing fabric, a normally insoluble binder composition confined substantially within the perimeters of the backing threads and that portion of the tufts which is in the plane of the backing, said binder material being so diffused in and around the individual fibers that a fiber lock, as opposed to a thread lock, of the tufts, is obtained.

5. An impregnated porous flexible single-plane backing pile fabric which consists of interwoven warp and weft backing threads, pile tufts having their tips free of impregnating material interlaced with said backing threads and having the pile bights projecting from the backing fabric, a normally insoluble binder composition confined substantially within the perimeters of the backing threads and that portion of the tufts which is in the plane of the backing, said binder material being in contact with a majority of the individual fibers of both the backing threads and pile tufts and not filling the interstices between the threads.

6. An impregnated porous flexible loosely woven single-plane backing pile fabric which consists of interwoven scoured warp and weft backing threads, pile tufts, the tips of which are free of impregnating material, looped around backing threads, a normally insoluble binder composition, confined substantially within the perimeter of the backing threads and that portion of the tufts which is in the plane of the backing, said binder material being so diffused in and around the individual fibres that a fibre lock, as opposed to a thread lock, is obtained and the interstices between the backing threads are not filled.

7. An impregnated porous single-plane backing V-pile fabric which consists of interwoven scoured warp and weft backing threads, pile tufts, having their tips free of impregnating material, looped around a single backing thread, a normally insoluble binder composition confined substantially within the perimeters of the backing threads and that portion of the tufts which is in the plane of the backing, said binder material being in contact with the majority of the individual fibres of both the backing and pile tufts.

8. An impregnated porous single-plane backing V-pile fabric which consists of interwoven warp and weft backing threads, pile tufts, having their tips free of impregnating material, looped around a single backing thread and having the pile bights projecting from the backing, a normally insoluble binder composition containing rubber confined substantially within the perimeters of the backing threads and that portion of the tufts which is in the plane of the back-

ing, said binder material being in contact with the majority of the individual fibres of both the backing and pile tufts.

9. An impregnated porous single-plane backing V-pile fabric which consists of interwoven scoured warp and weft backing threads, pile tufts, having tips which are free of impregnating material, looped around a single backing thread, a normally insoluble binder composition

containing rubber which is thoroughly diffused in and largely confined within said threads and locally to and in said pile tufts and that portion of the tuft which is in the plane of the backing threads so as to provide a discontinuous layer, whereby the interstices between the threads and tufts are not filled and the porosity as well as the textile feel is preserved.

GLEN S. HIERS.